

1

3,471,296

## SPIROCYCLIC QUATERNARY NITROGEN COMPOUNDS AS SILVER HALIDE SENSITIZERS

Harold Hückstadt, Cologne-Stammheim, Wilhelm Saleck, Schildgen/Bergedorf-Gladbach, and August Randolph and Erwin Ranz, Leverkusen, Germany, assignors to Agfa-Gevaert Aktiengesellschaft, Leverkusen, Germany, a corporation of Germany

No Drawing. Filed Dec. 16, 1966, Ser. No. 602,165  
Claims priority, application Germany, Dec. 28, 1965,

A 51,191  
Int. Cl. G03c 1/28

U.S. Cl. 96—107

6 Claims

## ABSTRACT OF THE DISCLOSURE

Photographic silver halide emulsions having their sensitivity increased by the addition of a compound having the formula:



in which X is a single chemical bond, a sulfur atom, a methylene group, a sulfonyl group or the quaternary nitrogen atom of a spirocyclically bound thiomorpholine ring, and A is any anion including a tosylate anion. Other sensitizers can be added as well as stabilizers.

The present invention relates to photographic silver halide emulsions chemically sensitized by the addition of heterocyclic sulfur compounds.

A number of methods have been described for improving the sensitivity of photographic silver halide emulsions other than by optical or spectral sensitization through the incorporation of certain sensitizing dyes in the emulsion. The incorporation of such dyes in the emulsion increases the optical or spectral range of sensitivity, and for this reason such dyes are commonly referred to as optical or spectral sensitizing dyes. Contrary to such optical or spectral sensitizers the so-called chemical sensitizers are believed to react with silver halide to form on the surface of the silver halide grain, sensitivity specks the chemical nature of which depends on the kind of the chemical sensitizer. The sensitivity of silver halide emulsions can be increased by chemical ripening or after-ripening during the preparation of the emulsion, by either prolonging the ripening time or by the addition of suitable substances such as compounds of noble metals or thiosulfate or other sulfur compounds. According to another method customarily employed the sensitivity of a photographic emulsion can be increased by the addition of development accelerators or chemical sensitizers to the emulsion, usually when it is completely ripened.

Suitable development accelerators are, for example, compounds containing onium groups (for example, quaternary ammonium or phosphonium and ternary sulfonium salts) and polyalkylene oxides and derivatives of polyalkylene oxides.

The process of chemical sensitization, however, reaches a limit beyond which further addition of sensitizing compounds or of prolonged digestion in the presence of a sensitizer, merely increases the undesired fog of the photographic emulsions.

In particular with respect to polyalkylene oxide sensitizers, many attempts have been made to increase the sensitizing action by modifying the chemical structure or by using them in combination with other compounds. However, in practice, none of these compounds com-

2

pletely meet the requirements as regards producing a satisfactory increase in sensitivity without concomitant increases in fog or poor keeping qualities.

The object of the present invention is to provide new chemical sensitizers which do not suffer the above disadvantages. Another object is to provide photographic silver halide emulsions having increased sensitivity and satisfactory keeping qualities.

We now have found that the sensitivity of an ordinary photographic silver halide emulsion can be substantially increased by incorporating therein spirocyclic, sulfur-containing quaternary salts of the following formula:



wherein

X=a single chemical bond, a sulfur atom, a methylene group, a sulfonyl group or the quaternary nitrogen atom of a spirocyclically bound thiomorpholine ring;

A=any anion, such as a halogen ion, preferably bromide, or a tosylate anion.

Particular utility is exhibited by the following compounds:



The spirocyclic quaternary salts to be used according to the invention may be prepared in known manner.

Thiomorpholine which can be prepared, for example, by the process described in German specification 1,104,513, is a particularly useful starting material.

The preparation of compound of the above general formula in which the group X is a methylene group, is described in detail below.

## COMPOUND I

## 6-azonia-9-sulfa-spiro-5,5-undecane bromide

5.15 g. (0.05 mol) of thiomorpholine and 11.5 g. (0.05 mol) of 1,5-dibromo-pentane are boiled under reflux for 4 hours with the addition of 7 g. of anhydrous potash in 50 ml. of n-butanol. At the end of this time, the product is filtered while hot from the potash. The desired compound crystallizes from the filtrate on cooling. It is separated by filtration under suction and recrystallized twice from methanol/ether. M.P. above 310° C. with decomposition.

5.7 g. of a white, finely crystalline powder is obtained.

## COMPOUND II

## 6-azonia-3,9-sulfa-spiro-5,5-undecane bromide-9-dioxide

23 g. of neutral thiomorpholine hydrochloride are dissolved in a mixture of 50 ml. of ethanol and 10 ml. of water, and after the addition of a small amount (about 15 droplets) of triethylamine as catalyst 19.8 g. of di-vinylsulfone are added dropwise. Reaction occurs under spontaneous heating and precipitation of colorless crystals. The reaction mixture is left standing over night and



The emulsions may also contain optical sensitizers such as the usual polymethine dyes such as neutrocyanines, basic or acid carbocyanines, rhodacyanines, hemicyanines, styryl dyes and oxonoles. Examples of these sensitizers have been described in the work by F. M. Hamer "The Cyanine Dyes and Related Compounds" (Interscience Publishers 1964).

The emulsions may be hardened in the usual manner, for example, using formaldehyde or halogen-substituted aldehyde which contain a carboxyl group, e.g., muco-bromic acid diketones, methane sulfonic acid ester and di-aldehydes.



10 tiser of the following formula (described in German patent No. 1,178,297)



10 Sample C: 480 mg. per liter of emulsion of ionic poly-alkylene oxide derivative of the following formula (according to German patent application A 50,595).

15 Sample D: 240 mg. per liter of emulsion of 6-azonia-9-sulfaspiro-[5,5]-undecane-bromide (Compound I) and 240 mg. per liter of emulsion of the polyethylene glycol phosphoric acid ester used in Sample B.

20 Sample E: 480 mg. per liter of emulsion of 6-azonia-9-sulfaspiro-[5,5]-undecane-bromide (Compound I) and 480 mg. per liter of emulsion of the polyethylene glycol phosphoric acid ester used with Sample B.

25 Sample F: 240 mg. per liter of emulsion of 6-azonia-9-sulfaspiro-[5,5]-undecane bromide (Compound I) and 240 mg. per liter of the chemical sensitizer already used with Sample C.

30 Sample G: 480 mg. of each of the compounds used in Sample F.

35 Sample H: 240 mg. per liter of emulsion of 6-azonia-9-sulfaspiro-[5,5]-undecane bromide (Compound I) and 240 mg. per liter of the chemical sensitizer used with Sample C and 480 g. per liter of emulsion of a thiazolidone stabilizer of the following formula (according to German patent specification 1,209,425):



40 Sample I: 240 mg. per liter of emulsion of 6-azonia-9-sulfaspiro-[5,5]-undecane bromide, 240 mg. of the polyethylene glycol phosphoric acid ester used with sample B per liter of emulsion and 480 mg. per liter of emulsion of the thiazolidone stabilizer of the following formula (according to German patent specification 1,209,425):



45 55 60 The samples were applied onto a cellulose acetate support, exposed and the dried layer developed as described in Example 1. The following table shows the sensitometric properties of the various emulsions:

TABLE 1

| Sample:         | 10 min. development |          |       | 20 min. development |          |      |
|-----------------|---------------------|----------|-------|---------------------|----------|------|
|                 | E                   | $\gamma$ | S     | E                   | $\gamma$ | S    |
| A..... Control. | 0.55                | 0.18     |       | Control.            | 1.10     | 0.17 |
| B..... +1.5°    | 0.37                | 0.13     | +1.5° | 0.80                | 0.14     |      |
| C..... +2.5°    | 0.48                | 0.09     | +2.0° | 0.80                | 0.13     |      |

## EXAMPLE 2

The same emulsion as in Example 1 was divided into 70 9 equal parts and the following compounds were added to the separate parts:

Sample A: Control sample—without additive  
Sample B: 480 mg. per liter of emulsion of the sensi- 75

TABLE 2

| Sample:         | 10 min. development |          |       | 20 min. development |          |      |
|-----------------|---------------------|----------|-------|---------------------|----------|------|
|                 | E                   | $\gamma$ | S     | E                   | $\gamma$ | S    |
| A..... Control. | 0.70                | 0.09     |       | Control.            | 1.20     | 0.10 |
| B..... +1.5°    | 0.80                | 0.08     | +1.5° | 1.20                | 0.14     |      |
| C..... +1.5°    | 0.80                | 0.11     | +1.5° | 1.25                | 0.15     |      |
| D..... +2.0°    | 0.75                | 0.11     | +3.0° | 1.20                | 0.15     |      |
| E..... +2.5°    | 0.85                | 0.12     | +2.0° | 1.25                | 0.20     |      |
| F..... +3.5°    | 0.80                | 0.12     | +3.0° | 1.25                | 0.19     |      |
| G..... +3.0°    | 0.85                | 0.16     | +3.0° | 1.15                | 0.19     |      |
| H..... +4.0°    | 0.80                | 0.11     | +4.5° | 1.15                | 0.19     |      |
| I..... +3.0°    | 0.75                | 0.11     | +3.5° | 1.25                | 0.17     |      |

7  
EXAMPLE 3

40 mg. per liter of the panchromatic sensitizer of the following formula



and 20 mg. per liter of the orthochromatic sensitizer of the following formula



were added to an emulsion as described in Example 1, 30 and the emulsion was then divided into four equal parts. The following compounds were added to the separate parts:

Sample A: Control sample—without additive

Sample B: 400 mg. per liter of emulsion of 6-azonia-9-sulfa-spiro-[5,5]-undecane bromide (Compound I)

Sample C: 240 mg. per liter of emulsion of 6-azonia-9-sulfa-spiro-[5,5]-undecane-bromide (Compound I) and 250 mg. per liter of emulsion of the chemical sensitizer used with Sample C of Example 2.

Sample D: 240 mg. per liter of emulsion of 6-azonia-9-sulfa-spiro-[5,5]-undecane bromide (Compound I) and 240 mg. per liter of emulsion of the compound of the type described in German patent specification 1,178,297 which was used in Example 2.

The samples were applied onto a cellulose acetate support and the dried layer exposed and developed as in Example 1.

TABLE 3

| Sample:         | 10 min. development |          |          | 20 min. development |          |   |
|-----------------|---------------------|----------|----------|---------------------|----------|---|
|                 | E                   | $\gamma$ | S        | E                   | $\gamma$ | S |
| A..... Control. | 0.65                | 0.12     | Control. | 1.10                | 0.05     |   |
| B..... +1.5°    | 0.65                | 0.03     | +2.0°    | 0.95                | 0.07     |   |
| C..... +2.5°    | 0.80                | 0.04     | +3.0°    | 1.25                | 0.09     |   |
| D..... +2.0°    | 0.70                | 0.04     | +2.0°    | 1.20                | 0.12     |   |

EXAMPLE 4

A silver iodobromide emulsion containing 6 mols percent of silver iodide was prepared according to common practice and divided into three parts ready for chemical ripening. The usual ripening additives, such as sulfur compounds, for example sodium thiosulfate and gold salts and after-ripening gelatin were added to the separate parts. In addition, the following compounds were added to the three parts.

Sample A: Control sample—without additive.

Sample B: 80 mg. per liter of emulsion of 6-azonia-9-sulfa-spiro-[5,5]-undecane bromide (Compound I).

Sample C: 160 mg. per liter of emulsion of 6-azonia-9-sulfa-spiro-[5,5]-undecane bromide (Compound I).

The after-ripening was completed and the samples applied onto a support of polyalkylene terephthalate. The dried layers were developed as described in Example 1.

TABLE 4

| Sample:         | 10 min. development |          |          | 20 min. development |          |   |
|-----------------|---------------------|----------|----------|---------------------|----------|---|
|                 | E                   | $\gamma$ | S        | E                   | $\gamma$ | S |
| A..... Control. | 0.75                | 0.10     | Control. | 0.95                | 0.16     |   |
| B..... +1.5°    | 0.70                | 0.12     | +3.0°    | 0.80                | 0.15     |   |
| C..... +2.0°    | 0.70                | 0.12     | +1.5°    | 0.90                | 0.19     |   |

EXAMPLE 5

The emulsion of Example 1 was divided into 4 equal parts and the following compounds were added to the 4 samples:

Sample A: Control sample—without additive.

Sample B: 240 mg. of compound II per liter of emulsion.

Sample C: 240 mg. per liter of emulsion of the sensitizer of Sample C of Example 2.

Sample D: 240 mg. per liter of emulsion of each of compound II and the sensitizer of Sample C.

The samples were applied onto a cellulose acetate support and the dried layer exposed and processed as described in Example 1.

TABLE 5

| Sample:         | 10 min. development |          |   |
|-----------------|---------------------|----------|---|
|                 | E                   | $\gamma$ | S |
| A..... Control. | 0.65                | 0.07     |   |
| B..... +2.5°    | 0.70                | 0.06     |   |
| C..... +2°      | 0.75                | 0.10     |   |
| D..... +3.5°    | 0.80                | 0.08     |   |

EXAMPLE 6

The emulsion of Example 1 was divided into 4 equal parts and the following compounds were added to the 4 samples:

Sample A: Control sample—without additive.

Sample B: 480 mg. of compound II per liter of emulsion.

Sample C: 480 mg. per liter of emulsion of the sensitizer of Sample C of Example 2.

Sample D: 480 mg. per liter of emulsion of each of compound II and the sensitizer of sample C of Example 2.

TABLE 6

| Sample:         | 10 min. development |          |   |
|-----------------|---------------------|----------|---|
|                 | E                   | $\gamma$ | S |
| A..... Control. | 0.57                | 0.07     |   |
| B..... +2.1°    | 0.63                | 0.08     |   |
| C..... +1.5°    | 0.65                | 0.09     |   |
| D..... +3.0°    | 0.70                | 0.12     |   |

We claim:

1. A light-sensitive material comprising at least one silver halide emulsion layer which contains a sensitivity-increasing amount of a chemical sensitizer of the following formula:



wherein

X represents a single chemical bond, a sulfur atom, a methylene group, a sulfonyl group or the quaternary

nitrogen atom of a spirocyclically bound thiomorpholine ring; and

A stands for an ion.

2. A light-sensitive material as defined in claim 1 in which the cation of the chemical sensitizer has the following formula:



3. A light-sensitive material as defined in claim 1 which in addition contains a sensitivity increasing amount of a chemical sensitizer of the polyethylene oxide series. 15

4. A light-sensitive material as defined in claim 3 in which the sensitizer of the polyethylene oxide series has the following formula:



wherein

R represents hydrogen or alkyl, acyl or phenyl and n an integer from 8 to 200. 25

5. A light-sensitive material as defined in claim 3 in

which the sensitizer of the polyethylene oxide series has the following formula:



wherein

R1 represents hydrogen or an alkylene oxide chain containing from 3 to 100 alkylene oxide units;

10 m is an integer from 3 to 100 and x is an integer from 1 to 10.

6. A light-sensitive material as defined in claim 1 which in addition contains a stabilizing amount of a thiazolidone stabilizer.

#### References Cited

##### UNITED STATES PATENTS

2,976,250 3/1961 Walford ----- 96—109 XR  
3,210,192 10/1965 Willems et al. ----- 96—110 XR

NORMAN G. TORCHIN, Primary Examiner

J. R. EVERETT, Assistant Examiner

U.S. Cl. X.R.

96—109